

E. O. POTTER.

Cartridge.

No 35,949.

Patented July 22, 1862.



Witnesses: { *John M. May*  
*Harry. McNamee.* } *Elam. O. Potter*  
By atty. *A. B. Strongham*

# UNITED STATES PATENT OFFICE.

ELAM O. POTTER, OF NEW YORK, N. Y.

## IMPROVEMENT IN CARTRIDGES.

*Specification forming part of Letters Patent No. 35,949, dated July 22, 1862.*

*To all whom it may concern :*

Be it known that I, ELAM O. POTTER, of the city, county, and State of New York, have invented a new and useful Improvement in Making Cartridges for Fire-Arms; and I do hereby declare the following to be a full, clear, and exact description of the same, reference being had to the accompanying drawings, making a part of this specification, in which—

Figure 1 represents a cartridge made of pressed powder, covered with collodion, and the cake of powder further secured to the ball by a belt of collodion. Fig. 2 represents, in section, the pressed powder, not incased, but secured to the ball by the collodion belt. Fig. 3 represents, in section, the collodion case and the belt both. Fig. 4 represents a cross section through the cartridge.

I am aware that a collodion covering has been used in a cartridge; and I am also aware that pressed powder for a cartridge has been used. I do not, therefore, claim either of these things.

There is a class of cartridges, however, viz., those in which a loose plug is inserted in the heel of the ball for the purpose of expanding it by the force of the explosion, with which it is difficult to use pressed powder, because the pressed powder cannot be united to the ball by any of the hitherto known ways without also so uniting or sticking the plug as to destroy its usefulness.

My invention is peculiarly applicable to the kind of cartridges above described, while for uniting pressed powder to any other kind of a ball it is very useful and valuable; and my invention consists in uniting pressed powder to a ball by running a collodion belt or zone around the joint or union between the powder and the ball, and extending over onto each

sufficiently far to firmly hold them together against the accidents of transportation or handling.

To enable others skilled in the art to make and use my invention, I will proceed to describe the same with reference to the drawings.

A represents an ordinary Minie ball, and B a cake of pressed powder united thereto by a belt or zone of collodion, *a*. In Figs. 1, 3, and 4 the cake of powder is represented as covered by collodion entirely, but as also secured by the belt or zone *a*, while in Fig. 2 the cake of pressed powder is held to the ball by the belt *a* alone, there being no covering to the pressed powder.

In some cartridges a plug of wood or other material is placed loosely in the cavity at the heel of the ball, and to unite pressed powder to such a ball, leaving the plug loose so that it may be driven up by the discharge to expand the heel of the ball, is a delicate operation. My plan of using the collodion belt or zone makes it perfectly practicable, and very easily accomplished. The plug being placed in the cavity of the ball, the cake of pressed powder is, or may be, brought into contact with the edges of the ball, leaving the plug loose, and while held there the film or belt of collodion is run around with a brush, and but a few moments are required to make them rigid enough to withstand all ordinary handling.

What I claim is—

Uniting solid or pressed powder to a ball by a belt or zone of collodion, in the manner and for the purpose substantially as described.

ELAM O. POTTER.

Witnesses:

A. B. STOUGHTON,  
HARRY W. PRICE.